

April 29, 1930.

P. S. McCANN

1,756,371

## CONTINUOUSLY LOADED CONDUCTOR

Filed July 6, 1927



Fig. 2.

INVENTOR  
PAUL S. McCANN  
BY J W Schmied  
ATTORNEY

## UNITED STATES PATENT OFFICE

PAUL S. McCANN, OF LA GRANGE, ILLINOIS, ASSIGNOR TO WESTERN ELECTRIC COMPANY, INCORPORATED, OF NEW YORK, N. Y., A CORPORATION OF NEW YORK

## CONTINUOUSLY-LOADED CONDUCTOR

Application filed July 6, 1927, Serial No. 203,732, and in Great Britain July 22, 1926.

This invention relates to loaded conductors and more particularly to conductors which are continuously loaded with a uniform covering of magnetic material.

Various magnetic materials have been proposed for this purpose, and they have been wound in the form of wire or tape around a conductor to form a continuous layer. Among the materials proposed are certain alloys which comprise metals of the magnetic group, usually nickel and iron in various proportions, with or without other ingredients. In order to obtain the necessary high permeability in alloys of this sort, it has been found to be necessary to subject the material to a specific and closely controlled heat treatment after it has been applied to the conductor.

It has been found that when the loading material is tight upon the conductor, its permeability after heat treatment is lower than when the material is less tight on the conductor. This effect may be due to stresses set up in the loading material due to the heat treatment. These stresses may be caused by unequal changes in the diameters of the conductor and the loading layer during the heat treatment whereby the loading material becomes stretched, or they may be ascribed to occasional weldings between the conductor and the loading material occurring when these are in intimate contact during the heat treatment, and giving rise to strains in the loading material when it is cooled down.

Various methods have been proposed for providing looseness during the heat treatment, for example, the operation of applying the loading material may be performed in such a manner as to form a loose winding. Another method is to interpose between the conductor and the loading material a spacing substance which may be burned off, vaporized, or otherwise removed during or just prior to the heat treatment. Other methods consist in providing a yielding layer between the conductor and the loading material or in de-

forming the conductor after the loading material has been wound in position so as to provide the required looseness. In accordance with another method the looseness is secured by twisting the loaded conductor before and during the heat treatment. 50

According to the present invention the loading material is placed directly upon the conductor before the final heat treatment and is subjected to a stretching process during or after the heat treatment, whereby the deleterious interaction between conductor and loading material may be overcome. The stretching may take place in whole or in part during the cooling stage of the heat treatment. The conductor may consist of a single copper wire, or as is more usually the case, may comprise a central copper wire around which are strained in known manner a plurality of flat copper tapes, and the loading material in the form of wire or tape is wound helically about the conductor without special care to secure looseness. The conductor may be stretched in any desirable manner to secure the necessary loosening of the loading material. 65 70

The invention will be described in connection with the accompanying drawing in which:

Fig. 1 shows a general arrangement of the apparatus for heat treating and stretching the loaded conductor; 75

Fig. 2 shows an alternate arrangement of such apparatus; and

Fig. 3 is a more detailed view of a gripping device for stretching the conductor. 80

Referring to Fig. 1, 10 and 11 indicate two furnaces which are in juxtaposition. These furnaces may be of any suitable type and heated in any desired manner. They are illustrated as being electric furnaces heated by coils diagrammatically shown at 12 and 13, respectively. The furnace 10 is longer than the furnace 11 and is maintained at a higher range. Instead of two furnaces, it is to be understood that a single furnace hav- 85 90

ing two zones maintained at different temperatures may be utilized or the heating means may be otherwise modified without departing from the scope of the invention.

5 Suitably supported within the furnaces 10 and 11 is a metallic tube 14 which communicates with a cooling tube 15. For a detailed description and illustration of the construction of the cooling tube 15 reference is 10 made to Patent No. 1,624,668, to F. S. Kochendorfer, issued April 12, 1927.

15 The strand 9 to be heat treated is in the form of a continuously loaded conductor and is fed from a supply reel (not shown) and 20 passed through a gripping device 18, and the tubes 14 and 15, and a second gripping device 19, and is then taken up on a storage reel (not shown).

25 For the sake of simplicity the drawings 20 only illustrate one heating tube and one cooling tube, but it is to be understood that in practice a plurality of tubes similar to the tube 14 may be mounted within the furnaces 10 and 11 and that a plurality of cooling tubes 15 may be utilized therewith. The gripping devices are designed to receive a 30 number of strands corresponding to the number of cooling tubes. By properly controlling the temperature of the furnaces and the 35 cooling tube as well as the speed with which the strand progresses therethrough the electrical characteristics of the loaded conductor and particularly the initial permeability of the loading material may be greatly improved.

40 In order to provide both a non-oxidizing and a non-reducing atmosphere in the heating tube 14, nitrogen under pressure is forced into the tube through a pipe 25, and in its 45 passage sweeps out any other gases that may be present in the tube.

45 The gripping devices 18 and 19 are identical in construction and are designed to firmly grip the conductor 9. The driving equipment for the gripping devices 18 and 19 consists of a motor 20, which may be of any suitable type and a shaft 21 suitably journaled in bearings and driven by the motor 20. A set 50 of gears 22 connects the driving shaft 21 with the gripping device 18 which thereby is driven at a constant predetermined speed. A similar set of gears 23 connects the driving shaft 21 to the gripping device 19, the ratio 55 of these gears being such that the device 19 is driven at a constant predetermined speed which is higher than that of device 18.

60 The construction of the devices 18 and 19 is shown more in detail in Fig. 3 and comprises a caterpillar mechanism consisting of 65 a pair of chains 31 and 32 carrying rubber gripping shoes 37 which are grooved to conform to the shape of the strand. The chains are mounted within a housing 30 upon sprockets 33, 34, 35 and 36, of which the three latter are mounted to rotate freely upon

shafts carried by the housing 30, whereas sprocket 33 is keyed or otherwise secured to a shaft 41 which is being driven through the set of gearing 22 or 23 shown in Fig. 1 from the motor 20. Secured to the sprocket 35 is 70 a gear 57 which meshes with a similar gear 56 secured to the sprocket 36 for driving the chains 31 and 32 in unison.

75 The strand 9 enters the housing 30, passes over a suitable stationary shoe 38, then between the rubber shoes 37-37, and leaves through a suitable opening 39 in the housing. The power supplied from the motor 20 to shaft 41 is transmitted by the sprocket wheel 33 through chain 31 to sprocket wheel 35 and gear 57, then over gear 56 to sprocket wheel 36, to chain 32, chains 31 and 32 thus move in unison and by exerting a tight grip on the strand 9 are able to exert a considerable pull on the strand.

80 To vary the pressure of the shoes 37-37 upon the strand 9, a stationary shoe 58 is suitably mounted between the sprockets 33 and 35 to engage the inside of the lower run of chain 31. Adjustably mounted in a housing 59 is 85 a shoe 60 which bears upon the inside of the upper run of chain 32. The shoe 60 is carried by two cams 61, each secured to a separate shaft 62, journaled in the housing 59, and each carrying a worm gear 63 which meshes with worms 64 secured upon a shaft 65, shaft 65 is supported in the housing 59 and at one end projects through the housing 30 and on its free end carries a crank 66. By turning the crank one way or the other the shoe 60 is 90 moved vertically up or down, to vary the pressure between the shoes 37-37, and the strand 9 to give the required traction.

95 Referring again to the general arrangement shown in Fig. 1, it is evident that on account of the tight grip of the caterpillar 18 on the strand 9, the strand enters the furnace 10 with a speed corresponding to the speed of the chains in the device 18. It is similarly evident that the strand leaves the cooling tube 15 with the speed of the chains in the caterpillar 19, which is higher than that of the chains in the caterpillar 18. The strand 9 is therefore subjected to a lengthwise pull 100 between the devices 18 and 19, which results in a stretching of the strand. This stretching has been found to be effective to increase the permeability of the loading material or to allow the permeability of the loading material to become fully developed by the heat treatment. This may be due to a reduction 105 in the diameter of the conducting core inside the layer of loading material caused by the stretching.

110 The arrangement for heating treating the conductor in accordance with this invention may be modified in accordance with that shown in Fig. 2 in which the parts corresponding to those shown in Fig. 1 are similarly numbered. The arrangement shown in 115

Fig. 2 departs from that shown in Fig. 1 only in the addition of a gripping device 17 driven through a set of gearing 24 from the motor 20, and acting on the strand 9 at a short distance beyond the device 19. In accordance with this arrangement the gearings 22, 23, and 24 may be dimensioned to impart speeds to the devices 18, 19, and 17, respectively, so that the stretching of the strand 9 may take place partly between devices 18 and 19 and partly between devices 19 and 17 or may be completely effected at either of these places.

The gripping devices 18, 19 and 17 have been described as being of the caterpillar type; however, it is possible within the scope of the invention to attain the desired stretching by the use of other devices, known in the art, which will firmly grip the wire and which may be driven at different speeds, it is furthermore not essential to the carrying out of the method that the devices 18, 19 and 17 are of similar construction or dimensions. The difference in speed imparted to the wire may furthermore be obtained by other means than the sets of gearings described and may be obtained by properly designing the devices 18, 19 and 17.

The method, as described, has a considerable advantage in that the loading material may be kept firmly on the conductor during the handling operations up to the heat treatment so that the conductor may be easily handled without damaging the loading. Moreover, in the present process the amount of stretching may be mechanically determined and may therefore be both adequate and uniform. A further advantage of the present process is that the loosening of the loading material may be effected during the drawing of the conductor through the furnace, and the necessity for a distinct process for this purpose is thus obviated.

If it, under certain circumstances, should be found convenient or desirable to carry out the stretching processes after the passage of the conductor through the furnaces, the arrangement shown in Fig. 2 and described above may be used, or the stretching process may be made a separate operation after that of the heat treatment. The loaded conductor is usually found to be in a more suitable condition for stretching or other deformation after heat treatment than before.

The invention is not limited to the methods and means of loosening the loading material which have been described. Any known and suitable means may be adapted for this purpose. The conductor may, for example, be rolled down or swaged either during or after the heat treatment to secure looseness or counteract the deleterious effect due to the heat treatment and thereby increase the permeability of the heat treated loaded conductor.

What is claimed is:

1. A method of improving a magnetic property of a continuously loaded conductor which has a non-adherent layer of a magnetic alloy about a central conductor which comprises subjecting the loaded conductor to a heat treatment and elongating the loaded conductor at any time after it enters said heat treatment. 70

2. A method of improving a magnetic property of a continuously loaded conductor which has a layer of magnetic material wound upon a central conducting core, which comprises subjecting the loaded conductor to a heating process and then to a cooling process 75 80 and stretching the loaded conductor at any time after it enters said heat treatment.

3. A continuous method of manufacturing a loaded conductor which comprises winding the loading material helically upon the conductor, then subjecting the loaded conductor to a heat treatment and elongating the loaded conductor at any time after it enters said heat treatment. 85

4. A continuous method of manufacturing a loaded conductor which comprises placing the loading material directly on the conductor, then elongating the loaded conductor and heat treating the loading material on the conductor during at least part of the elongating process. 90 95

5. A method of manufacturing a continuously loaded conductor which comprises placing the loading material directly on the conductor, then stretching the conductor and 100 heat treating the loading material during at least part of said stretching.

6. A method of loading a signaling conductor with a magnetic material which requires a heat treatment to give it a desired electrical characteristic, which comprises placing a layer of loading material upon the conductor and simultaneously stretching and heat treating said loaded conductor. 105

7. A method of loading a signaling conductor with magnetic material, which comprises placing a loading material tightly about the conductor, subjecting the loaded conductor to a heating and cooling treatment and stretching the conductor during at least 110 a part of said treatment to prevent deleterious interaction between the conductor and the loading material. 115

8. A method of producing a continuously loaded conductor which comprises surrounding a conductor with a layer of magnetic material, passing the loaded conductor through a heat treating apparatus in such a manner that the speed with which the conductor leaves said apparatus is higher than 120 that with which it enters. 125

9. A method of producing a continuously loaded conductor which comprises surrounding a conductor with a layer of magnetic material, passing the loaded conductor through 130

a plurality of gripping devices, and through a heat treating apparatus, the passage through at least one of said gripping devices taking place after commencement of the passage through said heat treating apparatus, the speed of one of said devices being higher than that of another of said devices whereby the loaded conductor is stretched to overcome deleterious interaction between the conductor and the loading material.

10 In witness whereof, I hereunto subscribe my name this 1st day of July, A. D. 1927.

PAUL S. McCANN.

15

20

25

30

35

40

45

50

55

60

65